

Feb. 2, 1932.

N. L. SNOW ET AL

1,843,790

BOILER CLEANER

Filed Nov. 21, 1927



*Norman L. Snow*  
*Samuel F. Cox*

*Attorneys*

*By William Alford Whiteman & Bellman*

## UNITED STATES PATENT OFFICE

NORMAN L. SNOW, OF NEW CANAAN, CONNECTICUT, AND SAMUEL F. COX, OF DETROIT, MICHIGAN, ASSIGNEES TO DIAMOND POWER SPECIALTY CORPORATION, OF DETROIT, MICHIGAN, A CORPORATION OF MICHIGAN

## BOILER CLEANER

Application filed November 21, 1927. Serial No. 234,784.

This invention relates to boiler cleaners and has particular reference to an improved blower element for structures of this character.

An object of this invention is to provide a blower element which will successfully meet in a practical manner, the very exacting requirements of articles of this character.

More particularly an object of this invention is to provide a blower element having 10 portions of different materials, the said materials having such characteristics that the various portions of the blower element will be particularly adapted to stand up under the deteriorating action to which the respective 15 portions are subjected.

Other objects and advantages of this invention will become apparent as the following description proceeds particularly when reference is had to the accompanying drawings wherein:

Figure 1 is a sectional view through a typical boiler showing a blower element associated therewith;

Figure 2 is a sectional view taken on the 25 line 2—2 of Figure 1;

Figure 3 is an elevational view of a blower element constructed in accordance with our invention;

Figure 4 is a sectional view through the 30 blower element taken on the line 4—4 of Figure 3; and

Figure 5 is a sectional view similar to Figure 4 showing a slightly modified form of blower element.

35 Referring now more particularly to the drawings wherein like reference characters designate corresponding parts throughout all views of the same, the reference character 10 designates a boiler of usual construction and 40 provided with the boiler tubes 11.

For the purposes of cleaning the tubes 11 of the boiler, there are provided the blower elements 12 which elements are arranged at suitably spaced points within the boiler 45 being supported in any desired manner, as for example by the bearings 13. The blower elements 12 may be mounted for rotation in a suitable head designated generally by the reference character 14 and may be supplied 50 with cleaning fluid through a suitable supply

pipe 15. All of this is of usual construction and forms no part of the present invention.

In certain locations of the blower elements or tubes 12 within the boiler, these elements must possess at least two distinct characteristics. The body of the blower element, that is the tube itself, must have enough structural rigidity, under the extremely high temperatures which are maintained at these certain locations within the boiler, to satisfactorily 60 resist the mechanical strains to which the blower element is subjected in service. The body of the element must be elastic or tough and yet it must not sag between its points of support when it is highly heated. Further, 65 the body of the element must be possessed of a high tensile strength and must be capable of resisting high temperatures for long periods of time and be capable of resisting sudden changes in temperature, since in operation when the cleaning fluid is admitted to these tubes their temperatures are rapidly 70 lowered by a considerable amount.

The second characteristic which a successful blower tube must possess, is that its surface be thoroughly resistant to the abrasive and scouring action of the furnace gases and ash incident to the operation of the boiler. The surface of these elements must be incapable of reacting with the chemical constituents of the furnace gases and must be particularly resistant to the action of sulphur which is contained in considerable amounts 80 in the furnace gases and ash.

Certain materials possess the first of the 85 above mentioned characteristics to a high degree but do not possess the other characteristic in a sufficient degree to render them thoroughly efficient and practical in the manufacture of the blower elements. Other materials possess the second characteristic to a high degree but do not possess the first characteristic to such a high degree. Our invention therefore consists in forming the blower element with a body portion formed of a 95 material possessing the requisite characteristics of the body of the element and in covering this body portion with a protective surface formed of a material possessing the second characteristic above outlined.

More particularly we have found that the body of the blower element may be successfully made of one of several different alloys. As an example we may form the body of the blower element 12 of a nickel manganese alloy and while it is obvious that the proportions of nickel and manganese may be varied to meet different requirements, we have found that when these materials are alloyed in the following proportion, the result is a material which efficiently meets the requirements of the first mentioned characteristic.

10 Nickel approximately 96  
15 Manganese approximately 4

As a second example we may form the body portion of the blower element of a nickel chromium iron alloy. Here also it is obvious that the proportions of the alloying metals may be varied to meet different requirements although we have found that when these metals are alloyed in the following proportions, they form a material which is thoroughly efficient in use.

25 Nickel 20 to 30  
Chromium 15 to 25  
Iron balance.

30 We have found that when the body of the blower element is formed of either of the above alloys, it possesses extremely high structural rigidity under the high temperatures to which it is subjected within the 35 boiler. Further the body of the element when formed of either of these alloys is sufficiently malleable to resist sudden changes in temperature and to resist the mechanical strains to which the blower element is subjected in operation.

40 For the surface of the blower element, we prefer to use a chrome iron alloy and these metals may be alloyed in any one of the three following proportions:

45 Chromium 11 to 14  
Carbon less than .50%, preferably under .25  
50 Silicon less than .50  
Manganese less than .50  
Sulphur less than .045  
Phosphorus less than .045  
55 Iron balance.

2 Chromium 16 to 19  
Carbon less than .25% preferably under .10  
60 Silicon .5 to 2.0% preferably .75 to 1.25  
Manganese less than .50  
Sulphur less than .045  
Phosphorus less than .045  
65 Iron balance.

|                         | 3.                   | Per cent |
|-------------------------|----------------------|----------|
| Chromium 26 to 30% -    | preferably 26 to 28  |          |
| Carbon less than .50% - | preferably under .25 | 70       |
| Silicon less than -     | .50                  |          |
| Manganese less than -   | .50                  |          |
| Sulphur less than -     | .045                 |          |
| Phosphorus less than -  | .045                 |          |
| Iron balance.           |                      | 75       |

We have found that when the surface of the blower element is formed of an alloy of chromium and iron in any of the proportions above specified, it will thoroughly resist the abrasive and scouring action of the furnace gases and ash incident to the operation of the boiler and will be particularly resistant to sulphur gases. Further the surface formed of this alloy possesses a high resistance to oxidation at high temperatures and is sufficiently malleable to resist the sudden temperature changes to which, as brought out before, the blower element is subjected.

The selection of the alloy to be used for the body of the element as well as the selection of the particular proportions to be used in the alloy for the surface of the element will be dependent upon the particular requirements of each installation. The alloys will be selected in accordance with the degree of malleability desired and the proportion of the ingredients in the two alloys may be varied to so reconcile the co-efficients of expansion of the two alloys that the composite tube will not be ruptured during its service. While we have suggested certain desired proportions in the alloys, it is obvious that many changes may be made to meet many different particular requirements.

In forming the tube of the several materials above mentioned, we may first form the inner tube or body portion 16 of the element 12 of relatively thick-walled material containing the metals specified, namely either nickel and manganese or nickel chromium and iron. The surface 17 of element 12 may then be formed of relatively thin material containing chromium and iron in the proportions desired and either shrunk or driven onto the body portion 16 of the element. The particular method of forming the composite element is not material since many methods known to those skilled in the art may be used.

After forming the composite tube or element the same may be drilled as at 18 for the reception of suitable nozzles 19.

As shown in Figure 4 of the drawings these nozzles 19 may have a body portion formed of one alloy and a surface formed of a second alloy similar to the element itself. If desired, however, the nozzle may be formed of a single material as illustrated in Figure 5 of the drawings and designated by the reference character 19'. If the nozzle is made of a single material, we prefer to make the same of

the chrome iron alloy having the same proportions as the surface of the blower element although it is to be understood that this nozzle may be made of either of the alloys as desired.

From the above, it will be apparent that we have formed a blower element which will efficiently withstand the hard usage to which the same is naturally subjected during the 10 operation of the boiler. That portion of the blower element, which is particularly subjected to the chemical action of the furnace gases, possesses those characteristics by which it may most efficiently withstand this chemical action while that portion of the blower element which must resist the strain incident to the heating and cooling of the element and the turning of the same during operation (if a rotatable blower element is used) possesses 15 those characteristics which will most successfully resist these strains.

While we have described with some particularity the preferred forms which our invention may assume, it is to be understood that 25 the embodiments described are for the purpose of illustration only and are not to be construed as definite of the limits to which our inventive idea may be put. We therefore reserve the right to make such changes in the 30 details of construction as will fall within the purview of the attached claims.

What we claim as our invention is:

1. In a soot blower cleaner tube, a body portion formed of an alloy containing nickel, 35 and a protective surface on said body portion formed of an alloy free from nickel.

2. A soot blower cleaner tube having a body portion formed of an alloy containing substantial quantities of nickel and having an 40 outer surface formed of an iron chromium alloy.

3. A soot blower cleaner tube having a body portion formed of an alloy containing over 45 20 per cent nickel and having an outer surface formed of an alloy containing substantial quantities of chromium and iron.

4. A soot blower cleaner tube having a body portion formed of an alloy containing substantial quantities of nickel and having an 50 outer surface formed of an alloy containing over 11 per cent chromium and over 50 per cent iron.

5. A soot blower cleaner tube having a body portion formed of an alloy containing substantial 55 quantities of nickel and having a surface formed of an alloy containing chromium from 11 to 30 per cent and iron from 68 to 88 per cent.

6. A soot blower cleaner tube having a body portion formed of one alloy and a surface formed of another alloy, one of said alloys containing substantial quantities of nickel and the other of said alloys containing substantial quantities 60 of chromium and iron and being free from nickel.

7. A soot blower cleaner tube having an outer surface formed of an iron chromium alloy and an inner body portion formed of a nickel chromium alloy.

8. A soot blower cleaner tube having an outer surface formed of an iron chromium alloy and an inner body portion formed of an alloy containing nickel 20 to 30 per cent and chromium 15 to 25 per cent.

9. A soot blower cleaner tube having an outer surface formed of an alloy containing chromium from 11 to 30 per cent and iron from 68 to 88 per cent and having a body portion formed of nickel 20 to 30 per cent, chromium 15 to 25 per cent and iron balance.

In testimony whereof I affix my signature.

SAMUEL F. COX.

In testimony whereof I affix my signature.

NORMAN L. SNOW.

85

90

95

100

105

110

115

120

125

130